

## UNITED STATES PATENT OFFICE

2,481,268

## CRANKCASE CONDITIONING OIL

C. Newbold Watson, Wynnewood, Pa., assignor to  
 Standard Oil Development Company, a corporation of Delaware

No Drawing. Application April 5, 1947,  
 Serial No. 739,658

1 Claim. (Cl. 252—33.4)

1

This invention relates to a crankcase conditioning oil and more particularly to a crankcase flushing and lubricating oil of the type employed for temporarily lubricating and cleansing the motors of automotive vehicles and internal combustion engines of comparable type.

It has been suggested in the prior art that certain cleansing compositions consisting partly or largely of suitable mineral oil base materials be used either in admixture with regular lubricating oil or by themselves for the purpose of cleansing the crankcase, cylinder walls, pistons, and other parts of carbonaceous, resinous, asphaltic, tarry and sludge deposits of various types and sources. It is desirable that such cleansing be accomplished during normal operation, and that the cleansing agent be also a lubricant during the period of cleansing.

The value of frequent engine cleansing is widely recognized, such cleansing being of particular utility in preventing clogging of oil systems, facilitating adequate lubrication and thereby preventing excessive wear, freeing frozen or stuck parts, such as valves, piston rings, and the like, and otherwise substantially improving the performance of internal combustion engines. The compositions used in the past, however, have not always been satisfactory, being deficient either in their cleansing capacity or their lubricating efficiency, or being corrosive in character, or being otherwise objectionable in many cases.

It is an object of my invention to supply an improved flushing composition which will be substantially free of the above-mentioned objections and to accomplish the foregoing by the use of readily available materials which are not excessive in cost and which can be used in a simple and efficient manner to cleanse internal combustion engines effectively without requiring disassembly and reassembly operations.

I have found that by using a composition comprising from 10 to 25% of an oil soluble metallo-organic base such as a metal petroleum sulfonate, or naphthenate mixed with from 25% to 40% of an aromatic solvent naphtha and from 40% to 50% of an aromatic extract obtained by solvent treatment of certain residual mineral oils, a very satisfactory conditioning oil may be obtained. Such a mixture as just described may be added to regular crankcase motor oil in proportions of 10% to 50% and used in the crankcase in the same way as regular lubricant. Preferably, such a mixture is used in lieu of, or in combination with a normal lubricating oil, for a suitable period, long enough to dissolve objectionable foreign

2

matter which accumulates on engine parts, and then is drained so that the regular lubricant may be replaced. Commonly a composition of this character mixed with lubricating oil will be used in automotive vehicles for about 50 to 500 miles depending upon the character of the vehicles and the amount and character of objectionable deposits.

As a specific example, a mixture of 11% by weight of sodium petroleum sulfonates, 1% of diethylene glycol, 3% of sodium naphthenates, 35% of an aromatic solvent naphtha having a boiling range of about 300 to 370° F., 5% of an extracted Coastal mineral oil (80 seconds viscosity at 210° F.) and 45% of an aromatic extract obtained by solvent treatment of residual lubricating stocks, was tested and found to be a very satisfactory composition. The solvent extract was prepared by phenol extraction of a Coastal naphthenic oil having a viscosity of about 500 S. S. U. at 100° F. Solvent naphtha was 95% aromatic and had a kauri-butanol value of 80.

The product just described was found to have the following physical characteristics:

|    |                          |      |
|----|--------------------------|------|
| 25 | Gravity, °API            | 17.0 |
|    | Flash, °F. (Closed cup)  | 115  |
|    | Viscosity SSU at 100° F. | 70.6 |
|    | Carbon residue, per cent | 4.20 |
|    | Ash, per cent            | 1.81 |

30 This material was added in a quantity of approximately 20% of the crankcase motor oil capacity together with 80% of regular lubricating oil. The engine was allowed to operate in normal service from 300 to 500 miles and thereafter the 35 crankcase was drained and regular motor oil re-installed.

In a further and more extensive test involving use of a large number of trucks in commercial service and operating under various conditions, 40 the product described above was found to be very effective in desludging automotive engines where the sludge was of the cold engine type. It is not as effective in removing high temperature varnish type sludge, although it has some utility for this 45 purpose. Cold engine sludges, however, are a major problem, involving about 80% of sludge troubles in engines of the automotive type.

In a competitive test conducted on a fleet of 50 dairy trucks, half of the trucks were treated with a well refined lubricating oil containing 20% of the above product and the other half were lubricated with a commercial heavy duty lubricating oil containing a detergent used in the prior art. After 5 months operation on these products, all 55 the engines were dismantled and examined.

Those operating on the heavy duty detergent oil were found to be very badly sludged, whereas those operating on the lubricating oil with 20% of my improved flushing oil incorporated therein were found to be exceptionally clean.

In another test, a Chevrolet taxicab fleet which had encountered severe engine sludging and particularly clogging of the rocker arm system, was lubricated with a 20% solution in standard lubricating oil of my improved flushing oil. Further sludging and oil system clogging were entirely eliminated in a test running over a period of a number of months.

Still another test was conducted to determine damage which might result from corrosion of bearings or clogging of oil screens or oil passages on the removal of sludge deposits. A 36-hour high temperature test on a standard Chevrolet engine was carried out according to the procedure described in U. S. Army specification 2-104B for the evaluation of heavy duty oils. The motor was operated for 36 hours continuously at a speed equivalent to 60 miles per hour and at an oil temperature maintained at 280° F. In this test my improved flushing oil was used in 30% concentration in standard lubricating oil. Bearing corrosion was found to be no greater than in the case of standard lubricating oil and engine cleanliness and mechanical conditions were found to be superior.

The improved performance of the flushing oil in comparison with competitive flushing solvents or compounds appears to be due to a combination of very effective solvency with the emulsifying and dispersing properties of a water-sensitive detergent soap. Solvents for carbonaceous products of fuels and oil decomposition in engine crankcases have been known in the prior art. However, when such deposits are in the form of an emulsion of water with lubricating oil, organic solvents have proved in the past to be relatively ineffective. This is due, apparently, to the protective action of the water emulsion. By combining effective solvency with an emulsifying dispersant the protective action of the emulsion component of the sludge appears to be overcome. The solvent naphtha serves to remove deposits from parts not normally contacted with effective amounts of an ordinary flushing oil, the naphtha tending to distill into the upper parts of an internal combustion engine in an automotive vehicle, for example. The solvent extract remains in the crankcase to serve as a solvent there.

As another example, a composition containing 25% by weight of an oil soluble metal sulfonate, specifically calcium sulfonate, mixed with 25% of aromatic solvent naphtha and 50% of aromatic extract obtained by the solvent treatment of naphthenic distillate, was found to be substantially equally satisfactory. My experiments indicate that various oil soluble sulfonates, such as those of calcium, barium, sodium and the like, as well as naphthenates of these and related metals, may be used successfully. In general, they will compose from 10 to 25% by weight of the flushing oil, although lesser or greater quantities may be used if desired. The aromatic solvent naphtha may have a boiling range between 250° and 450° F. and may be used in percentages ranging from 20 to 50% or more of the total composition. The other component, as suggested above, is preferably an aromatic extract obtained by conventional solvent treatment either of naphthenic distillate or residual lubricating stocks. Mixtures of extracts from these sources

may be used satisfactorily in any proportions, such materials comprising at least 25% and preferably making up 45 to 90% of the flushing or conditioning oil composition. Here again these limits are not critical, greater or lesser quantities being useful, but the ranges preferred are as indicated.

Flushing or conditioning oils prepared as above may be used without dilution and they are particularly effective cleansing agents when mildly heated. Preferably, however, they are used in standard lubricating oils over substantial periods of time permitting the solvent constituents sufficient time to loosen and dissolve the undesirable deposits in crankcases, valve compartments, piston ring grooves, and the like. Ordinarily they will be used in proportions of 10% to 50% of crankcase capacity in connection with lubricating oils of the type and grade approved for the particular engines being treated.

As will be obvious to those skilled in the art, various modifications may be made in the composition and other additives, such as corrosion inhibitors, antioxidants, extreme pressure agents, and the like, may be used in or in conjunction with flushing oils with or without lubricating oil dilution.

As suggested above, oil soluble metal naphthenates may be used to replace the oil soluble metal sulfonates wholly or in part. Thus a very satisfactory composition may include both sodium sulfonate and sodium naphthenate. For example, instead of using 10 to 25% sodium sulfonate, the composition may contain 0 to 25% sodium sulfonate and 25 to 0% of sodium naphthenate. A preferred range is from 3 to 15% sodium sulfonate and 2 to 10 percent sodium naphthenate. In lieu of either or both, the corresponding calcium salts may be used in like proportions. The total preferably amounts to at least about 10% based on the weight of the whole composition.

It is also desirable to include a small amount of a polyhydric alcohol, for example 0.1 to 5.0% of a glycol such as diethylene glycol. Ingredients of this character enhance the cleaning characteristics of the crankcase conditioning oil and contribute in some measure to its lubricating values. The solvents employed are as described above, and the composition so prepared is preferably used as an additive to a regular crankcase lubricating oil in proportions of 10 to 50%, based on the total finished lubricant, as previously described.

As a further specific example, a composition was prepared having the following composition:

|                    | Percent |
|--------------------|---------|
| Sodium sulfonate   | 10      |
| Sodium naphthenate | 3       |
| Diethylene glycol  | 1.2     |
| Water              | 1.0     |
| Solvent            | 84.8    |

The solvent consisted of about 40% aromatic solvent naphtha and about 60% aromatic extract, by solvent extraction, of residual mineral oils.

The composition just described may be added to conventional crankcase lubricating oils in various proportions as previously described, about 20% being considered a preferable proportion.

I claim:

A lubricating composition having cleansing properties consisting essentially of mineral base lubricating oil of internal combustion crankcase

lubricating grade, containing about 20% of a composition of the following approximate proportions by weight:

|                                                                                       | Percent |
|---------------------------------------------------------------------------------------|---------|
| Oil soluble sodium petroleum sulfonate                                                | 11      |
| Sodium naphthenate                                                                    | 3       |
| Diethylene glycol                                                                     | 1       |
| Aromatic solvent naphtha of boiling range<br>about 300° to 370° F                     | 35      |
| Mineral oil of about 80 S. S. U. viscosity at<br>210° F                               | 10      |
| Phenol extract of Coastal naphthenic oil of<br>about 500 S. S. U. viscosity at 100° F | 5       |
|                                                                                       | 45      |

## REFERENCES CITED

The following references are of record in the file of this patent:

## UNITED STATES PATENTS

| Number    | Name     | Date           |
|-----------|----------|----------------|
| 2,340,035 | Zimmer   | Jan. 25, 1944  |
| 2,262,926 | Edgar    | Nov. 18, 1941  |
| 2,214,634 | Dombrow  | Sept. 10, 1940 |
| 2,355,591 | Flaxman  | Aug. 8, 1944   |
| 2,415,353 | Johnston | Feb. 4, 1947   |

C. NEWBOLD WATSON.

15